

Aug. 26, 1952

P. H. JOHNSON ET AL

2,608,524

PROCESS FOR PRODUCING SUPERIOR MOTOR FUEL

Filed May 7, 1948



INVENTORS  
P. H. JOHNSON  
G. J. FORSETH

*Kudson and Young*

ATTORNEYS

## UNITED STATES PATENT OFFICE

2,608,524

PROCESS FOR PRODUCING SUPERIOR  
MOTOR FUEL

Paul Hilton Johnson, Bartlesville, Okla., and  
Glenn J. Forseth, Spring Valley, Wis., assignors  
to Phillips Petroleum Company, a corporation  
of Delaware

Application May 7, 1948, Serial No. 25,594

4. Claims. (Cl. 196—50)

1

This invention relates to a process for the manufacture of an improved motor fuel. In one of its more specific aspects, it relates to a process for the manufacture of motor fuels for internal combustion engines. In a preferred embodiment, this invention relates to the manufacture of an automotive gasoline fuel of superior road rating.

It is well known that in actual use, motor fuels of similar octane number will often give widely varying performance. The reason that the superior qualities of certain motor fuels do not show up in the laboratory is due to the inadequacy of the present testing methods. It is generally considered that a motor fuel which will knock the least is superior, and knocking is most apparent when an automobile is being accelerated and when the load on the engine is constantly changing. The knocking tendency of fuels as they are tested in the laboratory is determined with a motor operating at a relatively constant speed and at a constant load. Therefore, knocking data relative to acceleration and changing load are not obtained. Thus, the only entirely satisfactory testing method known at the present time is in stock automobile engines under conditions of actual "road rating test," i. e., driving the automobile and actually determining how the motor fuel acts under all road conditions. This type of test gives conclusive data as to the value of a motor fuel in actual service.

By such "road rating tests," it has been determined that the variation in performance of motor fuels of the same octane number is dependent to a great extent on the olefin content. It has been found that motor fuels containing substantial amounts of olefin hydrocarbons in the low boiling range and substantial amounts of aromatic, isoparaffinic, and/or naphthenic hydrocarbons in the high boiling range produce superior low and high speed performance in internal combustion engines of the type used in automobiles. Further, it has been found that the maximum boiling point of the olefinic components should not be in excess of about 250° F., the approximate mid-boiling point of gasoline motor fuel. The ideal fuel then, might be presumed to consist of approximately 50 per cent olefins boiling below 250° F. and 50 per cent aromatic, isoparaffinic, and/or naphthenic materials boiling above 250° F.

Broadly speaking, our invention comprises a single step catalytic cracking process for the manufacture of a superior "road rating" motor fuel. We have discovered that a mixture of

2

naphthenic naphtha and heavy gas oil contacted with a suitable dehydrogenation-cracking catalyst, such as bauxite, which will cause dehydrogenation, cracking, and aromatization, produces a superior automotive fuel.

In this specification, the term "naphthenic naphtha" as referred to means a mixture which includes a substantial proportion of those hydrocarbons known as naphthenes or cycloparaffins. By definition, naphtha is a mixture of low-boiling hydrocarbons and is a term well known to those skilled in the art. Also used in this specification is the term "gas oil." This may be either a virgin or synthetic gas oil which is a suitable cracking stock.

In accordance with our invention, a mixture of naphthenic naphtha comprised of cyclic paraffins having a boiling range of 250 to 400° F. and a gas oil comprised primarily of paraffins boiling in the range of 450 to 750° F. in a ratio of naphtha to gas oil of 1:5 to 5:1, however, preferably within the range of 1:2 to 2:1, is contacted under cracking conditions with a suitable dehydrogenation-cracking catalyst such as bauxite. The naphtha-gas oil mixture is charged to a suitable cracking unit at a temperature in the range of 800 to 1100° F., but preferably between 900 and 1050° F., a pressure in the range of 0 to 300 pounds per square inch, but preferably between 20 and 100 pounds per square inch, and a space velocity of from 0.5 to 5 liquid volumes of charge per volume of catalyst per hour. The total effluent from the cracking reaction is fractionated by suitable fractionation means to separate the normally gaseous materials, a superior road rating motor fuel, and heavy materials boiling above 400° F. which may be wholly or partially recycled as desired.

The action of the catalyst on the charge stock is primarily one of cracking, dehydrogenation, and aromatization. The gas oil by this treatment is cracked and dehydrogenated, thereby forming a predominance of olefins boiling below the mid-boiling point of gasoline. The naphthenic naphtha portion of the charge stock being inherently somewhat refractory is partially aromatized, thus giving both aromatics and naphthenes as products. The aforesaid fractionation of the total effluent produces a gasoline boiling range fraction of which the low-boiling half is comprised primarily of olefins and the higher-boiling half primarily of aromatics and naphthenes. This catalytic treatment of the naphthenic naphtha produces only very minor portions of paraffins and olefins.

Conventional catalytic cracking equipment is satisfactory for the operation of this invention. Suitable means should be provided for maintaining the desired temperatures, pressures, and other conditions required by the process in the various zones.

An object of this invention is to provide a process for manufacturing a superior motor fuel.

Another object is to provide a method for producing an improved motor fuel having a high 10 road rating at all speeds.

Another object of this invention is to provide a method for manufacturing an improved motor fuel which exhibits superior performance characteristics over the entire speed range, in 15 an internal combustion engine, particularly during periods of acceleration.

A further object is to provide a method for manufacturing a superior internal combustion engine fuel from naphthenic naphtha and heavy 20 gas oil.

A further object is to provide a method for producing a superior motor fuel by a catalytic process.

A further object is to provide a one step catalytic process for the manufacture of motor fuel.

A further object is to provide a method for manufacturing a superior road rating motor fuel by catalytically treating a mixture of naphthenic naphtha and gas oil.

Further objects and advantages of this invention will be apparent to one skilled in the art from the accompanying disclosure and discussion.

A better understanding of some of the many aspects of our invention may be had by referring to the attached schematic flow diagram in conjunction with the following discussion. It is understood that while this is representative in general of our process, various minor changes may be necessary in adapting it to the various conditions within the scope of the invention.

Naphthenic naphtha and steam (20 to 100 pounds per barrel of hydrocarbon feed) or other diluent are introduced into line 12 through lines 10 and 11, respectively, where they are admixed with heavy gas oil introduced through line 12. The hydrocarbon-diluent mixture passes via line 12 through preheater 13 and is introduced to catalytic cracking zone 14 at a temperature in the range of 800 to 1100° F. and a pressure in the range of 0 to 300 pounds per square inch. The mixture is contacted with a suitable catalyst, such as granular, calcined bauxite, which will cause dehydrogenation, cracking, and aromatization. Effluent from catalytic cracking means 14 is passed through line 15 to separation means 16. Light gases are removed through line 17, gasoline through line 18, water through line 19, and heavy residue through line 20. If desired, the heavy residue may be removed through the outlet in line 20 or recycled through lines 21 and 12 and preheater 13 to catalytic cracking means 14.

Advantages of this invention are illustrated by the following example. The reactants and their proportions, and other specific ingredients are presented as being typical and should not be construed to limit the invention unduly.

#### Example

All runs were made with a top catalyst temperature of 1020° F., a pressure of 85 pounds per square inch, and a space velocity of 1 volume of hydrocarbon per volume of catalyst per hour. Column 1 shows the properties of a gasoline produced by catalytically treating a gas oil boiling

5 in the range of 458 to 725° F. Column 2 shows the properties of a gasoline produced by treating a 250 to 400° F. straight-run naphthenic naphtha. Column 3 shows the properties of a blend of the 10 gasolines produced in runs 1 and 2, properties of which are shown in columns 1 and 2. Column 4 gives the properties of a gasoline produced by treating a 1:1 blend of the gas oil and naphtha used in runs 1 and 2.

| Column                  | 1    | 2    | 3    | 4    |
|-------------------------|------|------|------|------|
| ASTM Distillation, °F.: |      |      |      |      |
| IBP                     | 99   | 137  | 115  | 119  |
| 5% evap. 760 mm.        | 124  | 220  | 162  | 184  |
| 10%                     | 139  | 247  | 190  | 191  |
| 50%                     | 252  | 309  | 296  | 299  |
| 90%                     | 365  | 361  | 259  | 367  |
| EF                      | 402  | 408  | 396  | 408  |
| ASTM Octane Number:     |      |      |      |      |
| 0 cc. TEL               | 77.0 | 46.6 | 57.8 | 60.9 |
| 1 cc. TEL               | 79.5 | 56.0 | 65.5 | 67.8 |
| 3 cc. TEL               | 81.3 | 65.7 | 73.1 | 73.8 |
| Research Octane Number: |      |      |      |      |
| 0 cc. TEL               | 87.1 | 48.5 | 60.4 | 63.5 |
| 1 cc. TEL               | 90.5 | 55.9 | 69.1 | 71.1 |
| 3 cc. TEL               | 92.6 | 68.4 | 77.6 | 78.7 |
| API Gravity             |      |      |      |      |
| 56.6                    | 52.7 | 53.8 | 53.2 |      |
| Bromine Number          | 87   | 9    | 33   | 34   |

25 A comparison of the above data shows an improvement in the ASTM and Research octane number of the product gasoline from the combined treatment of the gas oil and naphthenic naphtha over that of the product of the separate treatment of the naphtha, or a combination of the products of the separate treatment of the gas oil and naphtha. The separate treatment of the gas oil provides the highest octane numbers of all, but it also shows a too high per cent of olefins boiling above 250° F. as indicated by the bromine number. This excess of olefins shows up disadvantageously in the road rating tests. Along with the improvement in octane numbers 35 of the gasoline product of the combined treatment is the improvement in road rating as may be shown by road tests. A further improvement is one of economics rather than in product. It is quite obvious that it would be much cheaper 40 to have only one catalytic treating unit rather than two for the treatment of the gas oil and naphthenic naphtha separately.

45 Although the process has been described and exemplified in terms of its preferred modifications, it is understood that various changes may be made without departing from the spirit and scope of the disclosure and of the claims.

We claim:

50 1. A process for the manufacture of a superior road rating motor fuel, which comprises forming a mixture of naphthenic naphtha boiling within a range of 250 to 400° F. and gas oil boiling within a range of 450 to 750° F., said naphthenic naphtha and gas oil being mixed in a ratio within the range of 1:5 to 5:1, contacting said mixture with a bauxite catalyst at a temperature in the range of 900 to 1050° F. and a pressure in the range of 0 to 300 pounds per square inch so as to produce an effluent, the gasoline fraction of which 55 consists of a low-boiling half comprising primarily olefins and a higher boiling half comprising primarily aromatics and naphthenes, and recovering said gasoline fraction as a product of the process.

60 2. A process for the manufacture of an improved road rating gasoline motor fuel, which comprises forming a mixture of naphthenic naphtha boiling within a range of 250 to 400° F., gas oil boiling within a range of 450 to 750° F., and an inert diluent, said naphthenic naphtha and

gas oil being mixed in a ratio within the range of 1:2 to 2:1, preheating said mixture to a temperature in the range of 900 to 1050° F., contacting said mixture with a bauxite catalyst at a pressure in the range of 0 to 300 pounds per square inch and a liquid space velocity of 0.5 to 5 volumes per volume of catalyst per hour so as to produce an effluent, the gasoline fraction of which consists of a low-boiling half comprising primarily olefins and a higher boiling half comprising primarily aromatics and naphthenes, and recovering said gasoline fraction as a product of the process.

3. A process for the manufacture of an improved road rating gasoline motor fuel, which comprises forming a mixture of naphthenic naphtha boiling in the range of 250 to 400° F., a virgin gas oil boiling in the range of 450 to 750° F., and steam diluent, said naphthenic naphtha and virgin gas oil being mixed in a ratio in the range of 1:2 to 2:1, preheating said mixture to a temperature in the range of 900 to 1050° F., contacting said mixture with a bauxite catalyst at a pressure in the range of 20 to 100 pounds per square inch and a liquid space velocity of 0.5 to 5 volumes per volume of catalyst per hour so as to produce an effluent, the gasoline fraction of which

5  
10

consists of a low-boiling half comprising primarily olefins and a higher boiling half comprising primarily aromatics and naphthenes, and recovering said gasoline fraction as a product of the process.

4. A process according to claim 1, wherein a steam diluent is used along with said naphthenic naphtha and said gas oil.

PAUL HILTON JOHNSON.  
GLENN J. FORSETH.

#### REFERENCES CITED

The following references are of record in the file of this patent:

#### UNITED STATES PATENTS

| Number    | Name            | Date           |
|-----------|-----------------|----------------|
| 2,283,854 | Friedman et al. | May 19, 1942   |
| 2,385,325 | Bailey          | Sept. 25, 1945 |
| 2,404,595 | Richker et al.  | July 23, 1946  |
| 2,406,112 | Schulze         | Aug. 20, 1946  |

#### OTHER REFERENCES

Chemical Constituents of Petroleum, by Sachanen (pages 197 and 200), Reinhold Pub. Corp., N. Y., 1945.